

May 1, 1945.

B. K. GREEN

2,374,862

COATING FOR PAPER

Filed June 19, 1942



Barrett K. Green  
Inventor

By *Carl Best*  
His Attorney

## UNITED STATES PATENT OFFICE

2,374,862

## COATING FOR PAPER

Barrett K. Green, Dayton, Ohio, assignor to The National Cash Register Company, Dayton, Ohio, a corporation of Maryland

Application June 19, 1942, Serial No. 447,681

16 Claims. (Cl. 106—137)

This invention relates to a coating for paper or similar web-like material, which coating will release, upon localized pressure being applied, included liquids for the purpose of marking a surface upon which the coating is overlaid.

The invention more particularly relates to a rupturable, elastic, solid film coating for paper, said film having dispersed profusely therein, at random, minute marking-liquid-containing cells of the so-called low-polarity or oil type, which are not affected adversely by atmospheric conditions causing hydrolysis, drying, or oxidation.

It has been known heretofore to make such coatings applied as a liquid which dries to a solid continuous phase with liquid inclusions therein, but said inclusions have been of a type which is more or less subject to change because of the atmospheric influences mentioned above.

Therefore, it is the principal object of this invention to provide a coating for paper that will form a rupturable solid film having profusely dispersed therein liquid inclusions of marking fluid of the low-polarity or oil type.

Another object of the invention is to provide a coating for paper which is applied as an emulsion, the continuous phase of which dries into a rupturable solid film having profusely dispersed therein colloidal sized liquid inclusions of the low-polarity or oil type, mentioned, which are resistant to change by atmospheric conditions.

The subject matter of this invention is an improvement over the types of coatings disclosed in my co-pending applications for United States Letters Patent, Serial No. 320,385, filed February 23, 1940, which issued as Patent No. 2,299,693 on October 20, 1942, and Serial No. 323,155, filed March 9, 1940, which issued as Patent No. 2,299,694 on October 20, 1942.

With these and incidental objects in view, the invention includes certain novel features, the essential elements of which are set forth in the appended claims and the preferred form or embodiment of which is hereinafter described in this specification with reference to the drawing.

## GENERAL DESCRIPTION

The novel coating consists of an emulsion having a continuous phase formed from a solid and a volatile liquid agent, and a low-polarity, low-viscosity, non-hygroscopic, dispersed phase preferably of the oil type, the two phases being separated by a strong inter-face structure. The emulsion so prepared is coated upon paper or web record material, and the continuous phase, which has in it the volatile agent, dries to a resilient rupturable solid film having within it the

discontinuous or dispersed phase in the form of minute liquid inclusions.

It is desirable that the coating produced be flexible and rupturable, and for that reason plasticizers are introduced into the continuous phase in the preferred form, although they may be omitted if conditions of use warrant. The discontinuous or dispersed phase of the coating may include, in addition to the low-polarity oil, selected pigments, staining liquids, or liquids which cause a stain by a chemical reaction or by contact with another surface.

The paper or web so coated may be used as a manifold sheet by laying the coated side of the sheet on which the marking is to be made, and causing pressure to be applied at selected localized points by means of a stylus, type, or other printing instrument, which pressures rupture the solid coating of the reverse side, releasing the dispersed liquid inclusions from their cells, allowing them to contact the undersheet or the coated sheet.

It is also within the scope of this invention to make a continuous phase having within it two types of such oil inclusions which are chemically separated from one another but which, when the stylus or printing member ruptures the coating locally, causes a local coalescing of the two types of cells, which, by chemical reaction, produces a localized stain, or to have the inclusions react with the paper upon which it is coated or upon chemicals in the paper or in the rupturable continuous phase. Such a film having heterogeneous cells is described in the Patent No. 2,299,693, to which reference has been made.

The preferred embodiment of the invention includes the forming of the liquid emulsion to be coated on the paper, said emulsion being made as follows:

| 40                              | External or continuous phase                               | Per cent |
|---------------------------------|------------------------------------------------------------|----------|
|                                 | Gelatin                                                    | 20       |
|                                 | Saponin                                                    | 1        |
| 45                              | Water                                                      | 79       |
|                                 | Total                                                      | 100      |
| Internal or discontinuous phase |                                                            |          |
| 50                              | Paraffin oil (viscosity 140-160 Saybolt at 100 degrees F.) | 47       |
|                                 | Chlorinated diphenyl (approximately 54% chlorine)          | 47       |
| 55                              | Tetra-methyl-diamino-diphenyl-phthalide                    | 2        |
|                                 | Thymol                                                     | 4        |

The internal and external phases are formed into an emulsion on a dried film basis in the proportions of 1/1. Other dyes, stains, or pigments may be substituted for the tetra-methyl-diamino-diphenyl-phthalide if desired.

A second emulsion having a methyl-cellulose external or continuous phase is made as follows:

*External or continuous phase*

|                                        | Per cent |
|----------------------------------------|----------|
| Methyl cellulose (extra low viscosity) | 10       |
| Water                                  | 90       |

*Internal or discontinuous phase*

|                                                   | Per cent |
|---------------------------------------------------|----------|
| Paraffin oil (viscosity 140-160 Saybolt)          | 49       |
| Chlorinated diphenyl (approximately 54% chlorine) | 49       |
| Tetra-methyl-diamino-diphenyl-phthalide           | 2        |

The internal and external phase ratio on a dry film basis is 1/2.

Examples of low-polarity and low-volatility liquids for the internal phase:

|                                |    |
|--------------------------------|----|
| Paraffin oil                   | 25 |
| Naphthenic oils                |    |
| Castor oil                     |    |
| Neatsfoot oil                  |    |
| Lard oil                       |    |
| Olive oil                      |    |
| Chlorinated diphenyls          | 30 |
| Tributyl phosphate             |    |
| Ethyl-phthalyl-ethyl-glycolate |    |

Examples of marking chemicals for the internal phase:

|                                                      |    |
|------------------------------------------------------|----|
| Reactive: Tetra - methyl-diamino- diphenyl-phthalide | 35 |
| Staining: Sudan IV                                   |    |
| Pigment: Carbon black                                |    |

Examples of emulsifying agents for the internal phase:

|             |    |
|-------------|----|
| Thymol      | 45 |
| Phytosterol |    |
| Cholesterol |    |

Examples of solid forming agents for the external phase:

|                  |    |
|------------------|----|
| Gelatin          | 50 |
| Casein           |    |
| Methyl cellulose |    |

Example of emulsifying agent for the external phase in addition to the solid forming substances mentioned:

Saponin

Example of drying agent for the external phase:

Water

The drawing shows the paper sheet 10 which is to be coated, having dried thereon the external phase 11 containing the low-polarity liquid inclusions 13. When the coated film side of the paper is placed in contact with an undersheet 14 and the uncoated side of the prepared sheet has localized pressure applied to it such as by a stylus 15, the rupturable film is broken, allowing the marking liquid to escape and mark the upper surface of the undersheet, as shown at 16. It is evident that the coalescing of the inclusions will make a visible mark on the paper which is coated or upon the film itself if reactive.

In making the emulsion, ordinary laboratory procedure is used. It is desirable to add the

proposed internal phase of the emulsion to the external phase while agitating the external phase.

While the form of the invention herein shown and described is admirably adapted to fulfill the objects primarily stated, it is to be understood that it is not intended to confine the invention to the one form or embodiment herein disclosed, for it is susceptible of embodiment in various forms all coming within the scope of the claims which follow.

What is claimed is:

1. A liquid emulsion having a continuous phase which is a solution of a solid in a drying liquid, said solid being rupturable by marking pressures and having a discontinuous phase of a low-polarity oily liquid containing a marking chemical.

2. A liquid emulsion having a continuous phase which is a solution of a solid in an evaporable liquid dryable to a rupturable solid film and having a discontinuous phase of an oily marking chemical remaining as discrete liquid inclusions in the external phase when dried.

3. A liquid emulsion having a continuous phase which is a solution of a solid in an evaporable liquid dryable to a rupturable solid film and having a discontinuous phase of a low-polarity non-hygrosopic marking chemical remaining as discrete liquid inclusions in the external phase when dried.

4. A liquid emulsion having a continuous phase which is a solution of a solid in an evaporable liquid dryable to a rupturable solid film and having a discontinuous phase of an oily low-viscosity marking chemical remaining as discrete liquid inclusions in the external phase when dried.

5. A sensitized record material including a base sheet having thereon a rupturable solid continuous phase containing a profusion of droplets of a liquid discontinuous phase, said droplets being of an oily marking chemical.

6. A sensitized record material including a base sheet having thereon a rupturable solid continuous phase containing a profusion of droplets of a liquid discontinuous phase, said droplets being of an oily low-polarity non-volatile marking chemical.

7. A sensitized record material including a base sheet having thereon a rupturable solid continuous phase containing a profusion of droplets of a liquid discontinuous phase, said droplets being of an oily non-hygrosopic marking chemical.

8. A sensitized record material including a base sheet having thereon a rupturable solid continuous phase containing a profusion of droplets of a liquid discontinuous phase, said droplets being of an oily non-oxidizing marking chemical.

9. A manifold sheet comprising a base sheet and a rupturable solid coating on the base sheet having discrete liquid inclusions of an oily marking chemical profusely dispersed therein.

10. A manifold sheet comprising a base sheet and a rupturable solid coating on the base sheet having discrete liquid inclusions of a non-hygrosopic oily marking chemical profusely dispersed therein.

11. A manifold sheet comprising a base sheet and a rupturable solid coating on the base sheet having discrete liquid inclusions of a non-volatile oily marking chemical profusely dispersed therein.

12. A manifold sheet comprising a base sheet and a rupturable solid coating on the base sheet having discrete liquid inclusions of a non-oxidizing oily marking chemical profusely dispersed therein.

13. An emulsion coating for paper, consisting of a continuous phase of a rupturable solid gelatin

film containing discrete oily marking liquid inclusions of low polarity.

14. An emulsion coating for paper, consisting of a continuous phase of a rupturable solid methylcellulose containing discrete oily marking liquid inclusions of low polarity.

15. An emulsion coating for paper, consisting of a continuous phase of a rupturable solid casein

containing discrete oily marking liquid inclusions of low polarity.

16. An emulsion coating for paper, consisting of a continuous phase of a rupturable solid containing discrete liquid inclusions of paraffin oil, a marking fluid, and chlorinated diphenyl.

BARRETT K. GREEN.